

April 24, 1928.

C. VANZETTI

1,667,642

METHOD FOR PREVENTION OF CRACKING OF CASTINGS

Filed Sept. 22, 1925



Inventor:

Carlo Vanzetti

By *Luise Vanzetti*  
Attorney.

## UNITED STATES PATENT OFFICE.

CARLO VANZETTI, OF MILAN, ITALY.

## METHOD FOR PREVENTION OF CRACKING OF CASTINGS.

Application filed September 22, 1925, Serial No. 57,961, and in Italy September 23, 1924.

It is known that in almost all metals the dimensions of the castings obtained by casting the molten metal are less than the corresponding dimensions of the mold. In general, for cast iron, a contraction of 1% generally occurs, while for steel this contraction can vary from 1 to 3%. The molds in which metal is cast generally comprise earth or sand, and are filled with the melted metal in a liquid state. When the mold is filled, the metal commences to pass into a solid state and it is then that the contraction takes place. During this period of contraction it is natural that the mold must follow the successively decreasing dimensions of the casting, and this is particularly true in the case of the core or in the parts of the mold which remain under compression on account of the contraction. However, the mold of earth or sand is always slightly deformable either on account of its own composition or because, by means of suitable devices, empty spaces are left at the proper points which fill up before fusion with the more yielding and more flexible material. But it is also certain that at the moment of fusion, while all the metal is still liquid, the latter exerts a hydrostatic pressure on the surfaces of the mold which must be very resistant at that time.

Theoretically the mold for casting metal of high contraction must, therefore, be very resistant from the start in order to resist the hydrostatic pressure of the metal, and must be readily deformable in the subsequent stage to permit the metal to contract as it cools.

If the mold is so strong as not to be deformable under the action of stresses produced by contraction, the casting would crack and crevices would be produced over its entire section, or else small fissures would be produced. The crevices or fissures would occur at the point of least resistance of the casting at the moment of rupture. For example it may happen that a steel casting breaks at its point of smallest section or, on the contrary, at its largest section, since at the moment of rupture the smallest section has already cooled considerably and can offer a resistance greater than that of larger sections which are still liquid or almost liquid. And it can also happen that the casting breaks at its smallest section as at the moment of rupture the largest sections have, for example, their external surface

already sufficiently cooled to enable the resistance of that section to be greater than the resistance of the smallest section.

It is also generally known that large castings, particularly if produced by metals having great contracting coefficients as for instance steel, can suffer great internal stresses during cooling down, if the molds do not move or adjust themselves in such manner that the contraction during cooling down can proceed regularly. This drawback is very important, if castings of such form are considered in which a part of the casting in one or two of the three dimensions is not equal to or proportional with the dimensions of the other parts, since in such case cracks or even total fractures take place. This particularly takes place quite often in quadrangular frame castings, tubes of greater diameter, etc.

This invention relates to a method, which enables the attainment of a general movement and contraction of the sand during the period of cooling down of the casting, and the examination and promotion of the contraction of the casting.

This contraction is obtained by any mechanical arrangement that can exert and regulate a sufficient pressure in all directions where an irregular contraction may cause a fracture or other flaw or flaws. This is accomplished by means of strong plates applied on the exterior part of the mold, and the pressure is applied on the plates by mechanical, hydraulic or other means. In this way the pressure can be regulated according to the time required, and the sand can completely move to accommodate the gradual contraction of the casting and even to precede it.

At the instant when the shrinking begins, a uniform pressure is applied on the mold. After the main contraction has taken place, the moment of the formation of cracks is present. These cracks arise in the parts of the casting which cannot resist with sufficient strength.

By careful examination of the shape of the casting and the location of risers one can determine beforehand the sections where cracks are most likely to occur. After several experiments one can follow accurately with the help of pyrometers located at predetermined places, the way in which the pressure and the sand motion should be adjusted.

The apparatus for carrying out this method depends upon the nature of the castings but for purposes of illustration several preferred forms of molds are shown on the 5 accompanying drawing in which:

Figure 1 is a cross-sectional view of a mold for casting a car frame,

Fig. 2 is a top view of the mold,

Fig. 3 is a sectional view of a mold for 10 casting a pipe, and

Fig. 4 is a sectional view of a modified form of mold shown in Fig. 3.

In the drawing there are indicated several 15 dimensions which are merely for the purpose of showing the large dimensions of the casting compared with the thickness.

The contraction or movement of the sand is accomplished by means of a pair of plates 1 and 1' and 2 and 2' disposed in the interior 20 of the frame 3 and respectively on opposite sides of the mold. The contraction or movement is accomplished by forcing screws 4 which are provided on a cross beam 5 and which move the plates. Nuts 6 (see Fig. 4), 25 can also be used, which are provided on the extremities of tie rods 6'. In each case these contracting plates produce a contraction and a movement of the sand following the contraction of the casting G, thus relieving 30 it of stresses. Thus the successful contraction of the casting is accomplished by means of the violent contraction and movement of the sand after having finished the step of actual casting.

25 I claim as my invention:

1. A mold for large castings, comprising a frame; and means in said frame for exert-

ing a pressure on the molding sand in the frame to thus force the sand to contract and move with the cooling of the casting.

2. A mold for large castings, comprising a frame; a plurality of plates provided in said frame; and means in said frame for actuating said plates in order to exert a pressure on the molding sand in the frame to thus force the sand to contract and move with the cooling of the casting.

3. A mold for large castings, comprising a frame; a plate provided on each side of said frame; and means in said frame for actuating said plates in order to exert a pressure on the molding sand in the frame to thus force the sand to contract and move with the cooling of the casting.

4. A mold for large castings, comprising a frame; a plurality of plates provided adjacent the sides of the frame; and screws threaded in said frame for actuating said plates in order to exert a pressure on the molding sand in the frame to thus force the sand to contract and move with the cooling of the casting.

5. A mold for large castings, comprising a frame; a plurality of plates provided adjacent the sides of the frame; screws threaded in said frame for actuating said plates in order to exert a pressure on the molding sand in the frame to thus force the sand to contract and move with the cooling of the casting; and cross beams for said screws.

65 In testimony whereof I affix my signature.

CARLO VANZETTI.